

# United States Patent [19]

Okamoto et al.

[11] 3,865,678

[45] Feb. 11, 1975

[54] SUEDE-LIKE RAISED WOVEN FABRIC AND  
PROCESS FOR THE PREPARATION  
THEREOF

[75] Inventors: Miyoshi Okamoto, Osaka-fu;  
Shusuke Yoshida, Otsu; Tadashi  
Imai, Otsu; Tatsuo Watanabe, Otsu;  
Shinzo Nishikaku, Kusatsu, all of  
Japan

[73] Assignee: Toray Industries, Inc., Tokyo, Japan

[22] Filed: Mar. 7, 1973

[21] Appl. No.: 338,962

[30] Foreign Application Priority Data

Mar 7, 1972 Japan ..... 47-22766  
Apr. 25, 1972 Japan ..... 47-40901

[52] U.S. Cl. .... 161/67, 161/172, 161/175,  
161/176, 161/181, 161/DIG. 2, 139/35,  
139/37, 139/392, 264/174

[51] Int. Cl. .... B29d 27/00, D04h 1/64

[58] Field of Search .... 264/174, 161/172, 175,  
161/176, 181, DIG. 2, 62, 64, 67; 139/392,  
35, 37

Primary Examiner—William J. Van Balen

[57]

## ABSTRACT

A suede-like raised woven fabric having raised fibers on the surface thereof; consisting mainly of a yarn or thread which consists of a bundle of extra-fine fibers (the monofilament denier of which is 0.0001 – 0.4 d). The preparation of the fabric comprises weaving, using as weft said yarn and using as warp a yarn having a coil-like crimp or a coil-like potential crimp capacity, in the organization of the woven fabric except for the raised portion, which consists of an elastic polymer dispersed and adhered in a fibrous state, and/or as fine pieces of film throughout the said fabric. Said fabric has a high density of suede-like naps, has excellent pilling resistance and, wrinkle resistance, feel, and is suitable for apparel.

[56] References Cited

### UNITED STATES PATENTS

3,705,226 12/1972 Okamoto et al. .... 161/67

50 Claims, 28 Drawing Figures





Fig. 1



Fig. 2



Fig. 3



Fig. 5

PATENTED FEB 11 1975

3,865,678

SHEET 2 OF 9

(80 X)

Fig. 4A



Fig. 4B



Fig. 4C



PATENTED FEB 11 1975

3,865,678

SHEET 3 OF 9

(240 X)



Fig. 4D

(800 X)



Fig. 4F

(800 X)



Fig. 4E

(2400 X)



Fig. 4G

PATENTED FEB 11 1975

3,865,678

SHEET 4 OF 9

(240 X)



Fig. 4H

(800 X)



Fig. 4J

(800 X)



Fig. 4I

(2400 X)



Fig. 4K

PATENTED FEB 11 1975

3,865,678

SHEET 5 OF 9

(240 X)



Fig. 4L

(800 X)



Fig. 4M

Fig. 4N



(240 X)



Fig. 4O

(2400 X)



Fig. 4P



PATENTED FEB 11 1975

3,865,678

SHEET 7 OF 9



*Fig. 8*



*Fig. 9*

PATENTED FEB 11 1975

3,865,678

SHEET 8 OF 9





Fig. 12



Fig. 13

## SUEDE-LIKE RAISED WOVEN FABRIC AND PROCESS FOR THE PREPARATION THEREOF

### BACKGROUND OF THE INVENTION

The present invention relates to a raised woven fabric whose surface is covered with extra-fine fibers having a suede-like touch, appearance and feel, and to a process for the preparation thereof.

Heretofore, raised woven fabrics consisting of extra fine fibers whose denier is below 0.8 d have been known. However, these conventional raised woven fabrics have had drawbacks in that they have poor pilling resistance. Additionally, they are in a blanket-like state which tends to encourage a loss of uniformity of organization ("loosing"); they are poor in wrinkle resistance and in hand feel; their color tone is light and they look whitish. Of these drawbacks, the occurrence of pills is a phenomenon that is inherent in a woven fabric of fine denier fibers. The finer the fiber constituting a fabric becomes, the smaller the apparent Young's modulus becomes, and the more entangled is a raised fabric woven therefrom. This is a drawback which has not been overcome by hitherto known antipilling means. For example, when a hitherto known anti-pilling method is employed, comprising lowering the tenacity of the fiber which constitutes the fabric in order to make the fabric anti-pilling, it is true that the pilling resistance is increased to some extent, but since the tenacity of the fabric per se is weak, the fabric becomes apt to break and cannot endure actual use. Further, the raised fibers become apt to fall off, with the result that the commercial value of the fabric is lost.

On the other hand, an artificial leather obtained by the process of impregnating a high molecular weight elastomer in a needle-punched non-woven felt using a special multi-core composite fiber or mix spun fiber to dissolve and remove a polymer component constituting said multi-core composite fiber or mix spun fiber, and then raising the surface, and a raised fabric consisting of a knitted or woven fabric which consists of said special multi-core composite fiber. Such technology is disclosed in the U.S. Pat. No. 3,705,226, to Okamoto et al., assigned to the assignee hereof.

However, said conventional artificial leather having a suede-like feel has many remarkably excellent points, but in some uses it has some drawbacks in that it does not have sufficiently satisfactory performance for use as apparel in respect to softness, drapeability, tenacity, tear strength, shape of wrinkle and uniformity of thickness, due to the properties of the non-woven fabric and the high molecular elastomer constituting the artificial leather. Because such artificial leather requires complicated processes such as needle punching and impregnation of the high molecular weight elastomer in manufacturing it, it requires strict quality control of the manufacturing steps followed in producing such artificial leather having fixed properties and performances. Needled felt has a disadvantage in that it is difficult to produce thin needled felt and when said felt is sliced to make it thin (for example 0.4 mm), its strength, especially its tear strength, is remarkably lowered.

On the other hand, a raised fabric consisting of a knitted or woven fabric has drawbacks in that when said composite fiber or mix spun fiber is used, by removal of one component of the polymer constituting said fiber, coarse spaces are formed in said knitted or woven fabric (lowering the density of the woven orga-

nization or woven configuration), and the woven organization cannot be covered enough with raised fibers. Moreover, because the lowering of balance between length and breadth concurrently with loosing among the woven organization and the change into fine fiber becomes remarkable, there is a drawback that the mechanical properties as a fabric become insufficient, the condition of the raised fibers is poor, occurrence of pills is remarkable and only a coarse raised bad fabric can be obtained.

### SUMMARY OF THE INVENTION

15 The present invention is the result of strenuous studies to produce a suede-like raised woven fabric free from the aforesaid drawbacks, having pliant raised fibers and a high density of the raised fibers.

20 An object of the present invention is to provide a raised woven fabric whose raised fibers are formed by a bundle of extra-fine fibers, having a high density of woven organization and being excellent in pilling resistance and feel, and to a process for the preparation thereof.

25 Another object of the present invention is to provide a raised woven fabric having a feel possessed by ordinary puffy knitted or woven fabrics in spite of using said bundle of fine fibers, and concurrently having an excellent surface condition of raised fibers, the same as that possessed by conventional natural suede leather.

30 Still another object of the present invention is to provide a raised woven fabric having excellent pilling resistance and having characteristics like those of suede leather, for example, reversible finger marks and feel, especially a thin raised fabric for apparel, and to provide a process for the preparation thereof.

35 The present invention attempts to attain the aforesaid various objects.

40 Primarily, the raised woven fabric of the present invention consists of a suede-like raised fabric which consists of a woven fabric, raised fibers covering the surface of said woven fabric and an elastic polymer impregnated throughout said woven fabric dispersing and

45 adhering in a dotted arrangement and in a fibrous condition, or as fine pieces of film. Said woven fabric consists of a yarn or thread the monofilament denier of which consists of a bundle of extra fine fibers being in the range of 0.0001 - 0.4 denier as weft yarns, and a 50 yarn having a coil-like crimp or a coil-like crimp capacity the total denier of which is 50 - 300 denier as warp yarns, where said raised fibers consist mainly of said extra fine fibers constituting the weft of the woven fabric.

55 The process for the preparation of the present invention consists of the following main steps.



A is the step of weaving into a woven fabric a yarn, consisting of an "islands-in-sea" type composite fiber in which the core components, the monofilament denier of which is 0.0001 - 0.4 d, are surrounded by another component (a sea component) or a mix spun fiber as weft; and weft yarns having a coil-like crimp or capable of developing a coil-like crimp.

B-I is the step of removing the sea component of the west.

B-II is the step of raising the surface of the woven fabric ((in this case, the "surface" is the rich side of the islands-in-sea type fiber)).

C is the step of impregnating a solution or emulsion of an elastic polymer into the woven fabric throughout the fabric at a predetermined concentration or, as a special case, coating said solution or emulsion on the back surface ((the poor side of islands-in-sea type fiber)) of the woven fabric, coagulating or drying and solidifying said solution or emulsion to apply said elastic polymer in a dotted configuration, in a fibrous condition, or as fine pieces of film.

D is the step of napping by rubbing the surface of the woven fabric with an appropriate material such as Emery (paper, cloth) or a grindstone and

X is the step of developing the crimp of the warp. This step X may be practiced at any stage after Step B-I, however, unless this step is performed, the product of the present invention cannot be obtained since this is an indispensable step.

B-I and B-II may be reversed with each other; however, the performance of step B-I before Step B-II is preferred.

The sequence of steps of A → B-II → C → B-I → D (+X) (the process steps of FIG. 13) is possible, but by performing the step C before the step B-I, the binding power between the fiber and the binder becomes small, and pilling resistance is somewhat inferior. However, lustrous good naps are formed. The raised woven fabric obtained by the foregoing structures and processes has the following characteristics:

## CHARACTERISTICS OF THE WOVEN FABRIC OF THE PRESENT INVENTION

1. Pilling resistance is excellent.
  2. It has good drapeability, being soft.
  3. Length and breadth of the fabric are balanced and it has no anisotropy.
  4. A smooth touch and appearance just like that of suede.
  5. It is unlikely to wrinkle, and wrinkles are unlikely to remain.
  6. Various kinds of woven fabrics having various thicknesses, ranging from thin fabrics to thick fabrics, may be made.
  7. Despite its use of extra-fine fibers, it has strong tenacity.
  8. Finger-marks appear.
  9. The raised fibers are reversible, having anisotropy.
  10. The raised fibers, being lustrous, tend to become uniform and parallel.
  11. It is easy to sew.
  12. Despite its being a woven fabric, the woven organization, i.e. the thread and yarn configurations, is unlikely to be visible, and it has an appearance like that of suede, or of a high class non-woven fabric.

13. The raised fibers are quite dense.
  14. Fallen fibers are few.
  15. Loosening is low and no fraying is likely.
  16. It has a warm feeling when worn.
  17. It has good uniformity of thickness.

Because of these characteristics, the raised woven fabric of the present invention splendidly overcomes drawbacks which we have heretofore been unable to overcome, as shown in the following comparative tables 1, 2 and 3.

### Comparative Table 1

|    | Conventional raised fabric                                                                                                                               | Product of the present invention                                                                                                                                            |
|----|----------------------------------------------------------------------------------------------------------------------------------------------------------|-----------------------------------------------------------------------------------------------------------------------------------------------------------------------------|
| 20 | Pilling resistance is poor.<br>Surface touch is rough.<br>Density of raised fibers is coarse.<br>Finger marks do not appear.<br>There are fallen fibers. | Pilling resistance is excellent.<br>It is pliant, having a smooth touch.<br>Density of raised fibers is quite dense.<br>Finger marks appear.<br>There are no fallen fibers. |
| 25 | Drapeability is poor.<br>Woven organization is conspicuous.<br>Raised fibers are not like those of suede.                                                | Drapeability is excellent.<br>Woven organization is unlikely to be seen.<br>It has an appearance like that of suede.                                                        |
| 30 |                                                                                                                                                          |                                                                                                                                                                             |

Comparative Table 2

|    |                                                                                                                                                             |                                                                                                                                   |
|----|-------------------------------------------------------------------------------------------------------------------------------------------------------------|-----------------------------------------------------------------------------------------------------------------------------------|
| 35 | Electro-static flocking goods                                                                                                                               | Product of the present invention                                                                                                  |
|    | Touch is rough.<br>Firm feel.<br>Poor in drapeability.<br>Finger marks do not appear.<br>There are restrictive limits to the length of the raised fibers.   | It has a suede touch.<br>Soft feel.<br>Excellent in drapeability.<br>Finger marks appear.<br>Length of raised fibers is optional. |
| 40 | Raised fibers have no luster.                                                                                                                               | Raised fibers have luster.                                                                                                        |
| 45 | It is likely to be wrinkled.<br>Raised fibers are uniform, having no variation.                                                                             | It is unlikely to be wrinkled.<br>Appearance is like that of natural suede.                                                       |
| 50 | It has a rubber-like feeling.<br>Curls tend to be brought about by dry cleaning. Dimension of a sewn good is apt to be crooked.<br>Shape stability is poor. | It has no rubber-like feeling.<br>Curls are hardly brought about by dry cleaning.<br>Shape stability is good.                     |

Comparative Table 3

|    | Extra fine materials                                                                                                                | Product of the present invention                                                                                                                   |
|----|-------------------------------------------------------------------------------------------------------------------------------------|----------------------------------------------------------------------------------------------------------------------------------------------------|
| 60 | <p>Pilling resistance is poor.</p> <p>Loosening tends to be brought about.</p> <p>Balance between warp and weft is not uniform.</p> | <p>Pilling resistance is excellent through use of a special anti-pilling method.</p>                                                               |
| 65 | <p>It is likely to be wrinkled.</p> <p>Raised fibers fall off.</p>                                                                  | <p>There is no loosening through use of a crimp developed yarn as warp.</p> <p>Balance is uniform through use of a special anti-pilling agent.</p> |

Comparative Table 3-Continued

| Extra fine materials                                                 | Product of the present invention                                                    |
|----------------------------------------------------------------------|-------------------------------------------------------------------------------------|
| Raised fibers are entangled and finger marks are unlikely to appear. | It is unlikely to be wrinkled.                                                      |
| Color is whitish.                                                    | Raised fibers do not fall off.<br>Finger marks appear.<br>Depth of color increases. |

In the present invention, other steps are frequently added, combined, or simultaneously carried out. In order to facilitate understanding of these other steps, flow sheets of these processing steps are shown in FIGS. 5 - 13. However, the main steps in the flow sheets do not change at all. That is, as shown in flow sheets 5 - 13, it may appear as if the steps of the present invention are many and complicated. However, the steps of the present invention actually are processes of a simple nature, with various additional steps added as shown in the flow sheets 5 - 13 as the need for their respective merits develops.

#### BRIEF DESCRIPTION OF THE DRAWINGS

FIG. 1 is a schematic illustration of a cross-section of an islands-in-sea type fiber;

FIG. 2 is a schematic cross-sectional view of one embodiment of the present invention.

FIG. 3 is a schematic cross-sectional view of one embodiment of bad raised fabric.

FIGS. 4 are scanning-type electron microscope photographs of three embodiments of the present invention;

FIGS. 4A, B and C being 80 X magnifications of a polyurethane impregnated fabric, a napped fabric, and a crimp developed (dyed) fabric, respectively;

FIGS. 4D and E being magnifications of the warp of the polyurethane impregnated fabric, 240 X and 800 X respectively;

FIGS. 4F and G being magnifications of the napped surface (weft) of the polyurethane impregnated fabric, 800 X and 2,400 X, respectively;

FIGS. 4H and I being magnifications of the warp of the napped fabric, 240 X and 800 X respectively;

FIGS. 4J and K being magnifications of the napped surface (weft) of the napped fabric, 800 X and 2,400 X respectively;

FIGS. 4L and M being magnifications of the warp of the crimp developed (dyed) fabric, 240 X and 800 X respectively;

FIGS. 4N, O and P being magnifications of the napped surface (weft) of the crimp developed (dyed) fabric, 240 X, 800 X, and 2,400 X respectively;

FIGS. 5 - 13 are process flow sheets of various embodiments of the present invention.

#### DESCRIPTION OF THE PREFERRED EMBODIMENTS

As the weft yarns constituting the woven fabric of the present invention, there is spun yarn (thread) or filamentary yarn containing a bundle of fine fibers the monofilament denier of which is 0.0001 - 0.4 d, preferably 0.05 - 0.17 d. When the denier is outside of the aforesaid range, the characteristics of a so-called suede-like raised woven fabric do not appear, and when the denier is less than 0.0001 d, because the weft is too fine, filament or fiber separability tends to be inferior,

and deep color does not tend to be obtained when the fabric is dyed. On the contrary, when the denier is more than 0.4 d, the feel of the raised woven fabric tends to become rough and a smooth touch tends not to be obtained.

Said spun yarn or filamentary yarn may be used as a single yarn also; however, it is especially desirable that said yarn be constituted as a twin yarn or a triple yarn since when said yarn is other than twin or triple yarn, 10 raised fibers in the state of downy hair or small loops are unlikely to be formed. Especially in the case of a single spun yarn, kinks tend to be formed upon spinning and the tenacity is low and undesirable. Accordingly, raised fibers of a raised fabric tend to fall out and 15 the length of the raised fibers tends to become great, and therefore fixation of the raised fibers is poor, rendering the single spun yarn inferior.

The weft used in the present invention is a 70 - 3000 denier (preferably 70 - 1000 denier) yarn containing 20 preferably more than 80% of a fiber of a type generating an extra-fine fiber such as a composite fiber of an islands-in-sea type, or a mix spun fiber containing 35 - 75% (preferably 40 - 60% by weight) of a core component forming a thin fiber. Expressed as a cotton count, 25 a 10 - 40 count is preferable.

FIG. 1 shows one of the cross-sections of an island-in-sea type fibers, where 1 designates the entire islands-in-sea type fiber, 2 designates the island component, and 3 designates the sea component. The denier of the entire islands-in-sea type fiber may be preferably 1 - 10 denier.

As examples of the core component constituting a bundle of fine fibers obtained from an islands-in-sea type composite fiber or a mix spun fiber, there are polyesters such as known homopolyesters (containing polyester ether) such as, for example, polyethylene terephthalate, polytrimethylene terephthalate, polytetramethylene terephthalate and polyethylene oxybenzoate; copolymers such as sodiumsulfoisophthalic acid, isophthalic acid and adipic acid; polyesters blended with various kinds of additives for the purposes of preventing static electricity, improving dyeability, preventing soil, retarding inflammability and preventing shrinking; and polyamides such as nylon 6, nylon 7, 40 nylon 11, nylon 12, nylon 66, nylon 610 (in this case "nylon" means polyamide), polyparaxylylene dodecane amide and polybiscyclohexylmethane dodecane amide or polyamides blended with various kinds of additives. Polyethylene terephthalate, polybutylene terephthalate or the copolymer thereof is preferable.

As the sheath or sea component (hereinafter referred to as the sea component) connecting these core (island) components, any compound will do insofar as it can be discharge shaped. Examples are polystyrene, polyethylene oxide, polyester and polyamide. Polystyrene or its copolymer is the most preferable. Alkaline-soluble polyester is the preferred type thereof.

The warp used in the present invention is a yarn or thread consisting of fibers having a coil-like crimp or a 60 yarn consisting of fibers capable of developing a coil-like crimp. Specifically, as a warp which can be used in the present invention, a false twisted processed yarn or composite potentially crimped yarn having a total denier of 50 - 300 d is especially preferable, by the use of which the thread entangle-pattern by weaving becomes inconspicuous, loosening is prevented and fixation of raised fibers is achieved. For the monofilament de-

nier (denier per filament) of the warp, 1 - 10 d (preferably 2 - 5 d) is ordinarily selected.

For the false twisted processed yarn, a fiber of the polyester, polyamide or polyacryl series, or the product obtained by combining at least two of these fibers, is used. A product made by false twisting a composite fiber of the polyester type series (example PET/TBT, two of different degree of polymerization PET PET//PET-copolymer), or a composite fiber, of the polyamide type series is preferable, and for the composite fiber, a fiber of the polyester series or the polyacryl series is preferable. If the island component and the warp thereof are both polyester, this is the most preferable combination.

Speaking as a whole, the spun yarn or filamentary yarn consisting of an islands-in-sea type composite fiber or a mix spun fiber constituting the weft must have such a woven configuration that 1 - 12 strands of said weft float toward the warp, as in, for example, 4-ply satin, 5-ply satin, etc, up to 12-ply satin or a modified woven fabric thereof. Unless a woven organization is taken in which 1-12 wefts float, the raising property is poor, the woven organization appears on the surface and even if it is a fabric in which a yarn having a large contracting power is used as the warp, a raised woven fabric of the type which is an object of the present invention is difficult to obtain.

However, the number of floating wefts is greatly affected by the denier ratio of the warp to the weft and is proportional thereto. When the number of floating wefts is small, they become difficult to raise, and the number of raised fibers becomes small; when the number of floating wefts is excessively large the raised fibers do not become fine and a plurality of large loops appear, which is not desirable (See FIG. 2). By having a proper number of floating wefts, the raising property of the fine fibers becomes excellent, the force restricting the warp is appropriate, large loops are not created by the raising process, and raised fibers in the form of downy hairs are obtained. Referring to the drawings, FIGS. 2 and 3 are cross-sectional schematic views of raised woven fabrics, wherein (4) is a warp consisting of crimped fibers, (5) is a weft consisting of a bundle of fine fibers, and (6), (7) and (8) are raised fibers. When a woven fabric having an appropriate number of floating wefts is subjected to raising processing, raised fibers (6) in the form of downy hairs consisting mainly of fine fibers of the weft (5) or raised fibers (7) in the form of small loops are formed, the weft (5) is mutually restricted with the warp (4), the weft does not float in the form of a large loop and a uniform suede-like woven fabric having a good cover of raised fibers is obtained (Fig. 2). (FIG.

On the other hand, when a woven fabric having an excessively large number of floating wefts is subjected to raising processing, because the restricting force of the warp (4) is weak, the weft (5) per se is pulled, becoming like a large loop, raised fibers in the form of downy hair or small loops of the fine fiber component of the weft (5) are difficult to obtain, and said woven fabric becomes a poor raised woven fabric having an appearance far from that of suede (FIGS. 3).

Specifically, when the denier ratio of the weft to the warp is Y and number of floating wefts is U, Y and U should satisfy the following relations:

a.  $30 \geq Y > 1.4$  and  $U = 1 - 7$   
or

b.  $1.4 > Y > 0.75$  and  $U = 3 - 12$

In the product of the present invention, a "cover factor" is important. This cover factor is defined by the following equation:

$$C = n / \sqrt{N}$$

where

C is the cover factor

N is the yarn count (cotton system) (before removing the sea component of the weft)

n is the number of yarns or threads (filaments) per inch.

This cover factor is important in the present invention and it should be within the range of preferably:

Toward weft  $19 > C_1 > 6.5$

Toward warp  $20 > C_2 > 6.0$  especially:

$17.0 > C_1 > 8.5$

$18.5 > C_2 > 8.0$

When  $C_1$  becomes more than 19 and  $C_2$  becomes more than 20, at the time of raising fibers, the fibers do not move and excellent raising cannot be carried out; and a raised woven fabric such as the product of the present invention cannot be obtained. Then  $C_1$  is less than 6.5, and  $C_2$  is less than 6.0, at the time of raising fibers loosening and breakage occur.

25 A fabric wherein  $U = 3 - 4$  and  $10.5 > Y > 1.5$  is most preferable.

On the other hand, when the denier ratio of the weft to the warp (Y) is more than 30, the fabric becomes a raised woven fabric in which the balance of length and breadth (warp and weft) is non-uniform, whereas when said denier ratio is less than 0.75, the density of the raised fibers by raising becomes small to say nothing of the imbalance of length and breadth (warp and weft) and a raised woven fabric which is an object of the present invention cannot be obtained.

The fabric having such a woven organization is then subjected to heat treatment and to a treatment for removing the sea component. The sequence of these 40 treatments is not particularly important, however, and the heat treatment and the treatment for removing the sea component may be carried out at the same time or the heat treatment and dyeing may be carried out at the same time.

45 Insofar as it occurs after removal of the sea component, the heat treatment may be carried out at any stage (time). However, after said removal, the earlier the heat treatment is carried out, the more a puffy and thick, good product is obtained.

50 Because crimp of the warp is unlikely to develop sufficiently before removal of the sea component, the heat treatment carried out at that time results in an inferior product. To a product not requiring much thickness, it is sufficient to carry out the crimp development and dyeing after the anti-pilling step.

55 It is preferable to carry out the heat treatment by hot water or steam at  $80^\circ - 120^\circ\text{C}$ ; however, where the heat treatment is carried out at the same time as the treatment for removing the sea component, it is carried out by the substance either dissolving or decomposing the sea component. For example, where the sea component is modified a polyester or polyethylene adipate easily soluble in an alkali solution, it is heat treated by hot alkaline water and the heat treatment and removal of the sea component are simultaneously carried out. Moreover, it is most efficient and economical to carry out the heat treatment and dyeing at the same time.

By this heat treatment, stress is brought about in a crimp generating direction of a false twisted yarn constituting the warp and the woven organization becomes dense, the thickness increases and the woven fabric becomes puffy. When using a potentially crimped composite fiber, crimp also develops by a heat treatment and the woven organization becomes dense. However, because a false twisted processed yarn is larger in crimp developing stress than the potentially crimped composite fiber, use of the false twisted processed yarn gives a better raised woven fabric having a more dense woven organization than that of potentially crimped composite fiber. Furthermore, in the case of PET fiber, 170° – 200°C heat-setting is preferable and heat-setting is most preferable after B-I and B-II.

If a fiber is contracted at a high ratio of 10 – 40% by heat treatment, the woven organization becomes dense or the density of raised fibers becomes good, which is preferable.

As a treatment for removing the sea component, dissolution with a solvent or removal by decomposition with heat or medicine is used. The solvent, medicine or temperature must be selected so as not to impart damage to the extent of losing the fiber form of the fine fibers. For example, where the fine fiber is polyethylene terephthalate and the sea component is nylon 6, it is preferable to use formic acid, hydrochloric acid and a calcium/methanol mixed solution; and where the fine fiber is polyethylene terephthalate or nylon 6 and the sea component is polystyrene, use of trichloroethylene and toluene is preferable. Again, in case the sea component is soluble in alkali, the use of hot alkali solution is preferable. The means and degree of the raising treatment may be properly selected in accordance with the contemplated uses and objects.

In the present invention it has been found that for raising the fibers, it is preferable to use various kinds of raising machines for wire cloth such as German-style, French-style, English-style and universal raising machines as well as Garnet or Emery raising machines.

At the time for raising, it is recommendable to carry out the raising at a stage before or after selectively removing by dissolution or mechanically removing at least one kind of polymer component constituting an extra fiber generating fiber in the organization of the woven fabric to make said fiber into a fine fiber, preferably after making said extra fine fiber generating fiber into a fine fiber. Further, we have found that it is recommendable to raise the fibers after carrying out various kinds of dyeing. In this case, a solution of anti-pilling reagent is preferably avoided. When fibers are raised after making said extra fine fiber generating type fiber into a fine fiber, because the degree of freedom of the extra fine fiber is great, said extra fine fiber tends to be raised. Because the opening properties of the extra fine fibers are increased by dyeing, the raising effect is great.

The raised woven fabric of the present invention is subjected to anti-pilling processing, about which mention will be made later. However, as another additional step, in an attempt to further advance fixation of the fixation of the raised fibers, it is possible to subject the fabric to a treatment for removing the sea component and a treatment for raising fibers. A woven fabric using as weft filaments obtained by mix spinning or mix weaving an islands-in-sea type composite fiber and/or a mix spun fiber and a fiber consisting of a polymer

whose softening point or melting point is lower than that of a polymer constituting said core (island) component (hereinafter referred to as a low melting point fiber), is treated, and thereafter said woven fabric is subjected to a heat treatment to soften or melt said low melting point fiber to connect the roots of the raised fibers with said woven fabric.

At this time, it is preferable from the viewpoint of processability and the characteristics of the product that the difference between the softening point or melting point between the core component and the low melting point fiber be more than 15°C, most preferably more than 25°C.

It is of course necessary to select the low melting point fiber in connection with the core component, and it is preferable in respect of dyeability that the two are polymers of the same series. For example, when the core component consists of polyester, for the polymer constituting said low melting point fiber, polyesters copolymerized with adipic acid, isophthalic acid, polyethylene glycol and diethylene glycol are optimum, and when the core component consists of polyamide, it is recommendable to use a copolymer of the polyamide series. However, said polymer is not particularly limited to a copolymer, but a homopolymer of the same series and a polymer of the different series will do insofar as they are low in softening point or melting point.

For lowering the melting point of the copolymer, a solvent may be used.

It is preferable that the ratio of the (multi-core) islands-in-sea type composite fiber and/or the mix spun fiber to the low melting point or low softening point fiber be within the following range.

$D/CA + D) \times 100 = 5 - 38\%$   
where A is the weight of the core component A, and D is the weight of the low melting point or low softening point fiber.

When the foregoing value exceeds 38%, the amount of fine fibers of raised fibers becomes small, and accordingly, the density of the raised fibers becomes low, while at the same time, the base tends to lack a smooth touch. On the contrary, when the value becomes less than 5%, fixation of the raised fibers decreases and the base fiber of said fabric tends to lack balance of feel and pilling resistance, and neither is preferable.

To such woven fabric, after being subjected to treatment for removing the sea component and to a raising temperature, a heating medium is used to soften or to melt at least a part of the low melting point fiber. For the heating method, it is preferable to bring a hot plate or hot roll into contact with the back surface where there are no raised fibers. The heating temperature should be a temperature higher than the softening point or melting point of the low melting point fiber and lower than the softening point of the core component and the base (substrate) sheet.

After passing through such heating step, the low melting point fiber which was constituting the raised portion softens or melts, a structure is formed in which this polymer connects the root of the raised fibers to the woven fabric, with the result that fixation of the raised fibers increases, and the pilling resistance and balance of feel between length and breadth (warp and weft) increase. Where the raised portions are connected by the softened or melted polymer by this heat treatment, because this polymer becomes very brittle by being exposed to a temperature higher than the soft-

ening point or melting point thereof, when the raised portions are buffed, raised and combed, this polymer may be simply removed.

Regardless whether such an additional step is adopted or not, a good raised woven fabric obtained by these steps in the present invention must be treated, without fail, in a proper concentration with at least one or more high molecular weight substances such as polyurethane, nitrile-butadiene rubber, polyvinyl chloride, polyvinyl acetate and polyamide or proper concentration for the purpose of improving feel, increasing stability of raised fibers or increasing balance between length and breadth (warp and weft) of the woven fabric.

As the method of imparting the high molecular weight substance, an indispensable step is the method of impregnating throughout the fabric a solution or emulsion dispersed liquid of this high molecular weight substance into said raised woven fabric, or applying said substance to the surface not raised, and thereafter drying or wet coagulating to solidify said substance.

The term "impregnating" the liquid throughout the fabric includes the processes of squeezing it by a nipping roll or a doctor-blade after the polymer-immersion into the fabric, but does not mean a coating of the liquid on the surface of the raised fabric.

A polymer may be coated onto the surface of the fabric or onto the back-side of the surface, but these two methods cannot readily achieve the objects of this invention. The former method has drawbacks such as unbalance of warp and weft of the fabric, fallen fibers, less-anti-pilling, and conspicuous woven organization (not-suede-like). The latter method has drawbacks such as less anti-pilling, no uniform raised fibers, rubber-like feel and less suede-like appearance. The former method is worse than the latter method, but all things considered, the above mentioned impregnation method is much better than either of the polymer-coating methods.

For a polyurethane which contains a polyether unit, a mixture of polyester and polyether having a hydroxyl terminal group (active hydrogen atoms) and polyurethane obtained from a polyester - polyether block copolymer is preferable.

However, it is necessary that an emulsion or organic solvent solution of polyurethane should have a concentration within the range of 1 - 9% by weight. Especially with the emulsion, the concentration should be 1 - 6% by weight, preferably about 2.0 - 3.0%; and with the organic solvent solution, a concentration within the range of 2.5 - 9.0% by weight, preferably about 4.0 - 6.0% by weight should be used. Although it depends upon the coagulating means after the impregnation, where the concentration of polyurethane becomes less than 1%, the feel of the obtained raised woven fabric becomes not greatly different from that of an untreated fabric; moreover, effects such as pilling resistance of the raised fabric and prevention of loss of the organization of the woven fabric are not adequate and the object of the present invention is not achieved. On the other hand, when the concentration exceeds 9.0% by weight, the surface forming raised fibers become like paper or scale, the ability of the raised fibers to form reversible anisotropic finger marks is not obtained by buffing, and when the degree of raising is made vigorous, loosing of the organization of the woven fabric or destruction of the organization is brought about, all of which are quite disagreeable results.

As the means for coagulating polyurethane, in the case of an organic solvent solution, these include dry solidifying and wet coagulation means, of which wet coagulation is the more preferable. Depending, however, upon the concentration, wet coagulation or dry solidifying may be used. In the case of an emulsion, there is available dry solidifying; and wet coagulation by an aqueous solution of a metal salt, a polar solvent and an aqueous solution thereof, an aqueous solution of an isomeric active agent, or an acidic aqueous solution. Dry solidifying is preferable.

By impregnation of polyurethane throughout the fabric, a thin polyurethane film is formed, surprisingly, on the surface of the raised woven fabric of extra fine fibers. The raised fibers fall down and become like paper, which is a phenomenon unseen in ordinary raised woven fabric of large denier. In a raised woven fabric consisting of a fiber of ordinary denier, the apparent Young's modulus of the raised fibers is large and the raised fibers hardly fall down with the impregnation of polyurethane. However, when the denier of raised fibers is thin and the apparent Young's modulus becomes small as in the present invention, the raised fibers remarkably tend to fall down with the impregnation of polyurethane.

Accordingly, in the present invention, it is necessary to buff the raised surface after impregnating an elastic polymer and drying the same, and by the way this buffing is carried out, it is possible to change the raised state, which process is called napping. It is found that by this process, a surface film of the polymer is removed, the polymer returns to the raised state, the raised fibers become shorter, and at the same time, more uniform, and the woven fabric becomes suede-like for the first time. Also the raised fibers become lustrous. Further, because it is possible to remove the impregnated elastic polymer which is undesirable for dyeing from among the raised fibers, the consequent dyeing is unlikely to become non-uniform and thus this napping is indispensable.

It is possible to incorporate carbon in an amount of 0.1 - 20% (based on the polymer) in the elastic polymer for the purpose of preventing poor dyeability, by which it is possible to decrease "color unbalance" by color mix. However, because carbon lowers wet friction dyeing fastness, it is preferable to use carbon in an amount as small as possible.

For napping, it is recommendable to buff the raised surface to the extent of not wearing away the interior of the organization of the woven fabric by using a sand roll or sand belt having 40 - 400 mesh (preferably 150 - 300 mesh sandpaper), sand cloth, Emery paper, or Emery cloth sand net.

When natural chalk mark properties and nap anisotropy are requested, buffing is carried out so as to disturb the natural direction of raised fibers on purpose. That is, the raised fibers are not permitted to fall down in one direction only, but are brushed transversely and then in an opposite direction so as to give anisotropy to a group of raised fine fibers on the surface which have become like paper. And where buffing is carried out in one direction only, the amount of raised fibers falling off by use becomes small. Therefore, it is preferable.

In the obtained raised woven fabric, on the base sheet (except the raised portion), said elastic polymer exists in a state of a plurality of fine film pieces, in a fibrous state, or in a dotted state as shown in FIG. 4. FIG. 4 is

a result of observation under a scanning-type electron microscope of a fabric impregnated with PU (polyurethane), a napped fabric and a crimp developed (dyed) fabric. Especially, because the roots of raised fibers are fixed by the elastic polymer, the raised fibers are prevented from falling off and surprisingly, piling resistance is imparted to the surface of the raised woven fabric. Immersing the polymer in the fabric using ultra-fine fiber is indispensable.

In the present invention, it is necessary to carry out 10 napping, i.e., another raising or buff processing after the elastic polymer is solidified. And in case there is some fuzz also on the back surface, it is recommendable to carry out buffing or burning of the fuzz. From the viewpoint of piling and stability of raised fibers, a 15 product of a superior quality is obtained when the elastic polymer is impregnated. Accordingly, impregnation is more preferable than coating.

Further, in the present invention, it is possible after dyeing or buffering to carry out water repellent, water resistant, soil resistant, anti-static, slime imparting, flame preventing and flame retardant treatments.

Especially in case of a woven fabric, it is necessary not to allow fuzz to appear on the back surface. However, a woven fabric in which extra fine fiber is used tends to produce fuzz on the back surface thereof. Accordingly, it is preferable to buff or shave the back surface after impregnation and drying. A method of burning fuzz on the back surface will do as well; however, strong brushing, shaving or buffing is preferable. It is preferable to carry out these operations weakly, lightly and at a high speed. By this, fuzz is removed and the surface of the raised woven fabric tends to become soft, and therefore, said removal of fuzz raises the commercial value of the product. When polyurethane is impregnated into the entire woven fabric after dyeing, it is preferable to so incorporate carbon and other coloring agents into polyurethane than they may become of the same series.

In order to make the finished product look like natural suede, it is necessary to carry out processing under such conditions that the thread entangle-pattern by weaving may not be seen or may not be conspicuously seen in advance in the raising step. In this connection, a false twisted processed yarn, or yarn-developing especially strong crimp, of a composite fiber developing strong potential crimp is effectively used as warp.

In order to prevent the thread entangle-pattern by weaving from being seen, it is especially preferable to use the weft threads by "woolen spinning", that is, its woolen type count should be:

or  $2/14$  -  $2/8$  (twin yarn)  
 $1/7$  -  $\frac{1}{4}$  (single yarn)

The thus obtained raised woven fabric of the present invention has a woven organization which is substantially the same as that of the woven organization of the woven fabric of the present invention.

- vention has the following characteristics:

  1. As compared with a conventional suede-like artificial leather based on a non-woven fabric of extra fine fiber, the raised woven fabric of the present invention is superior in pilling resistance, sewing properties, dyeability, color unbalance by color mix, softness of raised fibers, and is not inferior in a raised state.
  2. As compared with a conventional raised fabric consisting of extra fine fibers, the raised fabric of

the present invention is superior in pilling resistance, wrinkle resistance and setting properties, the falling off of a small quantity of raised fibers, and its feel is like that of leather.

3. It is possible to shorten the length of raised fibers and even when the length of the raised fibers is shortened, woven organization does not become conspicuous.
  4. Because the content of polyurethane is small, the adsorbed amount of a dyestuff at the time of dyeing by polyurethane is small and the dyeing efficiency is high. Accordingly, dyeing may be carried out at any stage either before or after raising.

Again, when a section of a raised woven fabric obtained by the present invention is observed under a microscope, it is found that polyurethane exists in dotted state, in a fibrous state, or as small pieces of thin film inside the organization of the woven fabric. However, polyurethane substantially hardly adheres to the organization of the raised fibers. The amount of adhered polyurethane to a fiber constituting the woven fabric is different. That is, said amount adhered to extra fine fibers constituting the raised fibers is different from that adhered to ordinary fiber, and it is considered that such state of adhered polyurethane is related to many characteristics of the present invention, especially to the increase of pilling resistance. In the raised woven fabric of the present invention, polyurethane acts as a sort of anti-pilling agent rather than as a conventional binder, having an entirely different function.

Because the raised woven fabric of the present invention has the aforesaid characteristics, it has many uses such as for suits, jumpers, blouses, pants, gloves, bags, upper garments, trousers, shirts, underwear, puffs, 5 chair covers and interiors. It is also possible to coat a polymer on this fabric. The raised woven fabric of the present invention may also be used efficiently after being bonded to or pasted together with various kinds of other materials. When these other materials are 0 woven fabrics, knitted fabrics or the same raised woven fabrics of the present invention, the bonding in a fibrous state and the net bonded state is excellent.

Hereinbelow, the present invention will be explained by reference to examples.

### EXAMPLE 1

As warp, a 150 denier/48 filament wooly (false twisted) yarn of polyethylene terephthalate was used and as weft, an islands-in-sea type composite fiber, whose island component consisted of a polymer which consisted mainly of polyethylene terephthalate and whose sea component consisted of a polymer which consisted mainly of polystyrene, was used. The particulars of the fiber used as weft were as follows:

|                                |               |
|--------------------------------|---------------|
| Number of islands              | 16            |
| Percentage of island component | 50%           |
| Percentage of sea component    | 50%           |
| Denier                         | 3.8 d         |
| Fiber length                   | 51 mm         |
| Number of crimp                | 12 mounts/in. |

These fibers were made into 20/2 S spun yarns. These yarns were used as warp and weft respectively, and woven into a 5-ply satin fabric so that the woven density might become 100 warps/in and 60 wefts/in. The denier ratio  $Y$  of the weft to the warp was 1.75 and the number of the floating wefts  $U$  was 4.

When this fabric was immersed in boiling water, the fabric contracted by about 14.1% longitudinally, by about 12.1% latitudinally, and by about 24.4% area contraction.

The contracted woven fabric was washed with trichloroethylene 5 times to remove the sea component of the weft, dyed in blue (Midnight color) with a dispersed dyestuff using a circular pressurizing dyeing machine, and then the dyed woven fabric was coated with an oiling agent and dried.

The dried woven fabric was passed through a French-type raising machine 7 times and a German-type raising machine 3 times (a total of 10 times), and thereafter passed through a shearing machine 2 times to obtain a raised woven fabric having excellent naps, whose threads entangle pattern by weaving was not conspicuous. When this raised woven fabric was subjected to brushing, the appearance became better.

Further, the raised woven fabric was immersed in and impregnated with a 5% DMF (dimethyl formamide) solution of polyurethane, a reaction product of methylene-bis-aniline (MBA), methylene-diphenyl-diisocyanate (MDI) and 75 parts of polyetherglycol and 25 parts of polyesterglycol. The impregnated fabric was squeezed, wet coagulated and dried. The amount of adhered polyurethane was 16.7 g/m<sup>2</sup>.

Subsequently, the dried fabric was subjected to finishing buffering 3 times by a belt sander buffering machine (sandpaper mesh No. 150).

The obtained buffed fabric was a suede-like raised woven fabric having better feel, short nice naps and balanced warp and weft without having naps in a state of scale, was excellent in pilling resistance and had a thickness of 0.82 mm. There was some fuzz on the back surface, which, however, could be beautifully removed by light buffering whereafter the fabric became soft suede having pilling resistance, excellent feel, and water-repellent without suffering loosening.

When a section of this suede was observed under a scanning-type electron microscope, it was confirmed that polyurethane in the state of a plurality of fine pieces of film or in a fibrous state adhered to the fiber of the fabric except for the raised portion.

The results of testing the physical properties of this suede were as follows:

## Comparative Example 1

When the raised woven fabric in Example 1 was immersed in and impregnated with a 13% DMF solution of polyurethane as in Example 1, wet coagulated and dried, the amount of adhered polyurethane was 41.6 g/m<sup>2</sup>.

Next, the dried fabric was subjected to finishing buffering as in Example 1. However, the surface forming raised fibers became like paper and the raised fabric became like scale.

The buffed fabric had poor feel and scale-like raised fibers, being a coarse fabric with rough surface touch, which eliminated its use for apparel.

When a section of this fabric was observed under a scanning-type electron microscope, it was observed that polyurethane in a state of film adhered to the entire fabric.

20

## EXAMPLE 2

A raised woven fabric processed by a method the same as that in Example 1 was impregnated with a 3% solution of polyurethane emulsion of the polyether series, dried and thereafter cured at 140°C for 10 minutes. The amount of adhered polyurethane was 7.9 g/m<sup>2</sup>.

Subsequently, the cured fabric was subjected to finishing buffering 4 times by a roller sander buffering machine (sandpaper mesh No. 180).

Said fabric became a high-class raised woven fabric having excellent feel and pilling resistance as well as suede-like naps the same as in Example 1.

Further, when a section of this fabric was observed under a scanning-type electron microscope, it was confirmed that polyurethane adhered to the fiber of the fabric except for the raised portion in a fibrous state or in a state of small pieces of thin film.

By varying the kind and concentration of polyurethane, the obtained fabrics were studied in detail and the results shown in Tables I, II, III and IV were obtained.

45

| Test                              |                    | Warp  | Weft |
|-----------------------------------|--------------------|-------|------|
| Density                           | No. / 25.4         | 118   | 85   |
| Thickness                         | mm                 |       |      |
| Weight                            | mm                 | 0.82  |      |
| Tear strength                     | g/m <sup>2</sup>   | 259   |      |
| Wrinkle resistant percentage      | kg                 | 4.60  | 2.77 |
| Decrease in weight by accelerator | %                  | 93.3  | 86.7 |
| Degree of bulkiness               | %                  | 2.2   |      |
| Rigidity                          | cm <sup>3</sup> /g | 3.20  |      |
| Tensile tenacity and elongation   | mm                 | 51    | 55   |
| Extension coefficient             | kg                 | 114.0 | 37.7 |
| Extension recovery percentage     | %                  | 73.0  | 36.5 |
| 1st time                          | %                  | 28.5  | 4.8  |
| 3rd time                          | %                  | 93.3  | 79.0 |
| 5th time                          | %                  | 91.1  | 68.4 |
| Washing shrinkage                 | %                  | 91.1  | 68.4 |
|                                   | %                  | 0.9   | 0.7  |

TABLE I

| Wet System (1)      |                   |                              |                                 |                       |                              |                       |                |          |
|---------------------|-------------------|------------------------------|---------------------------------|-----------------------|------------------------------|-----------------------|----------------|----------|
| Kind of PU (series) | Concentration (%) | Raised state                 | Pilling test ICI Method (grade) | Feel, Cantilever (mm) | Color unbalance by color mix | Directionality of nap | Depth of Color | Over-all |
| None                | 0                 | X (like blanket and flannel) | 1-2                             | 24                    | O                            | small                 | medium         | X        |
| PTHF 25/PCL 75      | 40                | X (like rubber sheet)        | —                               | —                     | X                            | —                     | —              | X        |
| do.                 | 30                | X (like rubber sheet)        | —                               | —                     | X                            | —                     | —              | X        |
| do.                 | 25                | X (like rubber sheet)        | —                               | —                     | X                            | —                     | —              | X        |
| do.                 | 18                | X (like rubber sheet)        | —                               | —                     | X                            | —                     | —              | X        |
| do.                 | 15                | X (like scale)               | —                               | 56                    | X                            | —                     | —              | X        |
| do.                 | 12                | X (like scale)               | —                               | 50                    | X                            | —                     | —              | X        |
| do.                 | 9                 | O                            | 5                               | 45                    | O                            | large                 | medium         | O        |
| do.                 | 7                 | O                            | 5                               | 37                    | O                            | large                 | medium         | O        |
| do.                 | 5                 | O                            | 5                               | 30                    | O                            | large                 | large          | O        |
| do.                 | 3                 | O                            | 5-4                             | 27                    | O                            | medium                | medium         | O        |
| PTHF 50/PCL 50      | 35                | X (like rubber sheet)        | —                               | —                     | X                            | —                     | —              | X        |
| do.                 | 30                | X (like rubber sheet)        | —                               | —                     | X                            | —                     | —              | X        |
| do.                 | 25                | X (like rubber sheet)        | —                               | —                     | X                            | —                     | —              | X        |
| do.                 | 20                | X (like rubber sheet)        | —                               | —                     | X                            | —                     | —              | X        |
| do.                 | 16                | X (like scale)               | —                               | 53                    | X                            | —                     | —              | X        |
| do.                 | 10                | X (like scale)               | —                               | 44                    | X                            | —                     | —              | X        |
| do.                 | 7                 | O                            | 5                               | 35                    | O                            | large                 | medium         | O        |
| do.                 | 5                 | O                            | 5                               | 29                    | O                            | large                 | large          | O        |
| do.                 | 2.5               | O                            | 5-4                             | 28                    | O                            | medium                | medium         | O        |
| do.                 | 2.0               | X (like blanket and flannel) | 3-2                             | 26                    | O                            | small                 | medium         | X        |
| PTHF 75/PCL 25      | 25                | X (like rubber sheet)        | —                               | —                     | X                            | —                     | —              | X        |
| do.                 | 18                | X (like rubber sheet)        | —                               | —                     | X                            | —                     | —              | X        |
| do.                 | 13                | X (like scale)               | —                               | 50                    | X                            | —                     | —              | X        |
| do.                 | 9                 | O                            | 5                               | 42                    | O                            | large                 | medium         | O        |
| do.                 | 7                 | O                            | 5                               | 36                    | O                            | large                 | medium         | O        |
| do.                 | 5                 | O                            | 5                               | 28                    | O                            | large                 | large          | O        |
| do.                 | 3                 | O                            | 5                               | 26                    | O                            | medium                | medium         | O        |
| do.                 | 1.5               | X (like blanket and flannel) | 3-2                             | 25                    | O                            | small                 | medium         | X        |

(For Method of Estimation for Tables I, II, III, and IV, see Page 46)

TABLE II

| Wet System (2)             |                   |                              |                                 |                       |                              |                       |                |          |
|----------------------------|-------------------|------------------------------|---------------------------------|-----------------------|------------------------------|-----------------------|----------------|----------|
| Kind of PU (series)        | Concentration (%) | Raised state                 | Pilling test ICI Method (grade) | Feel, Cantilever (mm) | Color unbalance by color mix | Directionality of nap | Depth of Color | Over-all |
| PTHF 100                   | 25                | X (like rubber sheet)        | —                               | —                     | X                            | —                     | —              | X        |
| do.                        | 20                | X (like rubber sheet)        | —                               | —                     | X                            | —                     | —              | X        |
| do.                        | 15                | X (like scale)               | —                               | 53                    | X                            | —                     | —              | X        |
| do.                        | 10                | X (like scale)               | —                               | 42                    | X                            | —                     | —              | X        |
| do.                        | 8                 | O                            | 5                               | 37                    | O                            | large                 | medium         | O        |
| do.                        | 6                 | O                            | 5                               | 30                    | O                            | large                 | large          | O        |
| do.                        | 4                 | O                            | 5                               | 27                    | O                            | large                 | large          | O        |
| do.                        | 2                 | X (like blanket and flannel) | 2-1                             | 25                    | O                            | small                 | medium         | X        |
| PPG 50/PCL 50              | 15                | X (like scale)               | —                               | 55                    | X                            | —                     | —              | X        |
| do.                        | 10                | X (like scale)               | —                               | 46                    | X                            | —                     | —              | X        |
| do.                        | 5                 | O                            | 5                               | 30                    | O                            | large                 | large          | O        |
| do.                        | 3                 | O                            | 5                               | 28                    | O                            | large                 | medium         | O        |
| PPG 75/PCL 25              | 10                | X (like scale)               | —                               | 45                    | X                            | —                     | —              | X        |
| do.                        | 5                 | O                            | 5                               | 29                    | O                            | large                 | large          | O        |
| do.                        | 2                 | X (like blanket and flannel) | 3-2                             | 26                    | O                            | small                 | medium         | X        |
| PPG 97/PEG 3               | 10                | X (like scale)               | —                               | 47                    | X                            | —                     | —              | X        |
| do.                        | 5                 | O                            | 5                               | 27                    | O                            | large                 | large          | O        |
| PPG 100                    | 10                | X (like scale)               | —                               | 45                    | X                            | —                     | —              | X        |
| do.                        | 5                 | O                            | 5                               | 26                    | O                            | large                 | large          | O        |
| PEA                        | 10                | X (like scale)               | —                               | 44                    | X                            | —                     | —              | X        |
| do.                        | 5                 | O                            | 5                               | 27                    | O                            | medium                | medium         | A        |
| conventional raised fabric | 0                 | Δ (touch is rough)           | 3-2                             | 30-35                 | O                            | small                 | small          | X        |

TABLE III

| Kind of PU<br>(series)               | Concen-<br>tration<br>(%) | Raised state          | Pilling test<br>ICI Method<br>(grade) | dry system (1)<br>Feel, Cantilever<br>(mm) | Color un-<br>balance by<br>color mix | Direction-<br>ality of nap | Depth of<br>Color | Over-all |
|--------------------------------------|---------------------------|-----------------------|---------------------------------------|--------------------------------------------|--------------------------------------|----------------------------|-------------------|----------|
| PTHF 50/PCL 50                       | 25                        | X (like rubber sheet) | —                                     | —                                          | X                                    | —                          | —                 | X        |
| do.                                  | 20                        | X (like rubber sheet) | —                                     | —                                          | X                                    | —                          | —                 | X        |
|                                      | 16                        | X (like rubber sheet) | —                                     | —                                          | X                                    | —                          | —                 | X        |
| do.                                  | 10                        | X (like rubber sheet) | —                                     | —                                          | X                                    | —                          | —                 | X        |
| do.                                  | 7                         | X (like scale)        | —                                     | 52                                         | X                                    | —                          | —                 | X        |
| do.                                  | 5                         | X (like scale)        | —                                     | 48                                         | X                                    | —                          | —                 | X        |
| do.                                  | 3                         | O                     | 5                                     | 36                                         | O                                    | Large                      | Large             | O        |
|                                      | 1.5                       | O                     | 5                                     | 31                                         | O                                    | Medium                     | Medium            | O        |
| PTHF 75/PCL 25                       | 25                        | X (like rubber sheet) | —                                     | —                                          | X                                    | —                          | —                 | X        |
| do.                                  | 15                        | X (like rubber sheet) | —                                     | —                                          | X                                    | —                          | —                 | X        |
| do.                                  | 12                        | X (like rubber sheet) | —                                     | —                                          | X                                    | —                          | —                 | X        |
| do.                                  | 9                         | X (like rubber sheet) | —                                     | —                                          | X                                    | —                          | —                 | X        |
| PTHF 75/PCL 25                       | 5                         | X (like scale)        | —                                     | 45                                         | X                                    | —                          | —                 | X        |
| do.                                  | 3                         | O                     | 5                                     | 33                                         | O                                    | Large                      | Large             | O        |
| do.                                  | 2                         | O                     | 5                                     | 30                                         | O                                    | Large                      | Large             | O        |
| do.                                  | 1                         | O                     | 5-4                                   | 28                                         | O                                    | Medium                     | Medium            | O        |
| Emulsion of the polyether series (1) | 40                        | X (like rubber sheet) | —                                     | —                                          | X                                    | —                          | —                 | X        |
| do.                                  | 20                        | X (like rubber sheet) | —                                     | —                                          | X                                    | —                          | —                 | X        |
| do.                                  | 10                        | X (like rubber sheet) | —                                     | —                                          | X                                    | —                          | —                 | X        |
| do.                                  | 5                         | X (like scale)        | —                                     | 75                                         | X                                    | —                          | —                 | X        |
| do.                                  | 3                         | O                     | 5                                     | 44                                         | O                                    | Large                      | Large             | O        |
| do.                                  | 1.5                       | O                     | 5                                     | 35                                         | O                                    | Medium                     | Medium            | O        |
| Emulsion of the polyether series (2) | 40                        | X (like rubber sheet) | —                                     | —                                          | X                                    | —                          | —                 | X        |
| do.                                  | 20                        | X (like rubber sheet) | —                                     | —                                          | X                                    | —                          | —                 | X        |
| do.                                  | 10                        | X (like rubber sheet) | —                                     | —                                          | X                                    | —                          | —                 | X        |
| Emulsion of the polyether series (2) | 8                         | X (like scale)        | —                                     | 75                                         | X                                    | —                          | —                 | X        |
| do.                                  | 5                         | X (like scale)        | —                                     | 73                                         | X                                    | —                          | —                 | X        |
| do.                                  | 2                         | O                     | 5                                     | 47                                         | O                                    | Large                      | Large             | O        |
| do.                                  | 1                         | O                     | 5-4                                   | 34                                         | O                                    | Medium                     | Medium            | O        |

Note: Emulsion of the polyether series

(1) "VONDIC 1010" C

(2) "VONDIC 1030"

C "VONDIC" is a trade name of Doinikkon Ink and Chemicals, Inc.

TABLE IV

| Kind of PU<br>(series)               | Concen-<br>tration<br>(%) | Raised state                 | Pilling test<br>ICI Method<br>(grade) | dry system (2)<br>Feel, Cantilever<br>(mm) | Color un-<br>balance by<br>color mix | Direction-<br>ality of nap | Depth of<br>Color | Over-all |
|--------------------------------------|---------------------------|------------------------------|---------------------------------------|--------------------------------------------|--------------------------------------|----------------------------|-------------------|----------|
| Emulsion of the polyether series (3) | 40                        | X (like rubber sheet)        | —                                     | —                                          | X                                    | —                          | —                 | X        |
| do.                                  | 20                        | X (like rubber sheet)        | —                                     | —                                          | X                                    | —                          | —                 | X        |
| do.                                  | 10                        | X (like scale)               | —                                     | 99                                         | X                                    | —                          | —                 | X        |
| do.                                  | 5                         | X (like scale)               | —                                     | 86                                         | X                                    | —                          | —                 | X        |
| do.                                  | 4                         | O                            | 5                                     | 50                                         | O                                    | Large                      | Medium            | O        |
| do.                                  | 3                         | O                            | 5                                     | 45                                         | O                                    | Large                      | Large             | O        |
| do.                                  | 2                         | O                            | 5                                     | 39                                         | O                                    | Large                      | Large             | O        |
| do.                                  | 1                         | O                            | 5-4                                   | 31                                         | O                                    | Medium                     | Medium            | O        |
|                                      | 0.5                       | X (like blanket and flannel) | 3-2                                   | 28                                         | O                                    | Small                      | Medium            | X        |
| Emulsion of the polyether series (4) | 45                        | X (like rubber sheet)        | —                                     | —                                          | X                                    | —                          | —                 | X        |
| do.                                  | 20                        | X (like rubber sheet)        | —                                     | —                                          | X                                    | —                          | —                 | X        |
| do.                                  | 15                        | X (like rubber sheet)        | —                                     | —                                          | X                                    | —                          | —                 | X        |

TABLE IV—Continued

| Kind of PU<br>(series)                     | Concen-<br>tration<br>(%) | Raised state                    | Pilling test<br>ICI Method<br>(grade) | dry system (2)<br>Feel, Cantilever<br>(mm) | Color un-<br>balance by<br>color mix | Direction-<br>ality of nap | Depth of<br>Color | Over-all |
|--------------------------------------------|---------------------------|---------------------------------|---------------------------------------|--------------------------------------------|--------------------------------------|----------------------------|-------------------|----------|
| Emulsion of<br>the polyether<br>series (4) | 9                         | X (like scale)                  | —                                     | 98                                         | X                                    | —                          | —                 | X        |
| do.                                        | 7                         | X (like scale)                  | —                                     | 92                                         | X                                    | —                          | —                 | X        |
| do.                                        | 5                         | X (like scale)                  | —                                     | 87                                         | X                                    | —                          | —                 | X        |
| do.                                        | 3                         | O                               | 5                                     | 48                                         | O                                    | Large                      | Large             | O        |
| do.                                        | 1                         | O                               | 5                                     | 33                                         | O                                    | Medium                     | Medium            | O        |
| do.                                        | 1.5                       | X (like blanket<br>and flannel) | 3-2                                   | 30                                         | O                                    | Small                      | Medium            | X        |

Note: Emulsion of the polyether series

(3) "VONDIC 1310"

(4) "VONDIC 1340"

"VONDIC" is a trade name of Doinikkon Ink and Chemicals, Inc.

## Method of estimation for Tables I, II, III, and IV:

|                 |                                            |
|-----------------|--------------------------------------------|
| 1. Raised state | Judged by naked eye                        |
| 2. Pilling test | ICI Method (JIS L 1076)                    |
| Grade           | Estimation                                 |
| 5               | Wherein piling hardly occurred             |
| 4               | Wherein piling occurred a little           |
| 3               | Wherein piling occurred considerably       |
| 2               | Wherein piling occurred greatly            |
| 1               | Wherein piling occurred remarkably greatly |

## 3. Feel Cantilever Method

On a board inclined by 45°, a sample was caused to slide and the distance between the stopped sample and the point contacting the slope was measured. For example, in the case of a sample as hard as iron, the value became infinity. The larger the numeral, the harder the sample. [ — in the Tables shows a self-evident hard sample of rubber quality not requiring measuring]

## 4. Color unbalance by color mix

— judged by naked eye

## 5. Directionality of Nap

Large — When one's hand is passed over a surface of a raised fabric having naps, the naps are equal along the direction one's hand passed over.

## 5. Directionality of Nap

Medium — When one's hand is passed over a surface of a raised fabric having naps, the naps are equal along the direction one's hand passed over, except for a portion.

Small — When one's hand is passed over a surface of a raised fabric having naps, the naps are not equal along the direction one's hand passed over.

## 6. Depth of Color

Large — When one's hand is passed over a surface of a raised fabric having naps, in the opposite direction to the naps, the depth of color changes and increases.

Medium — When one's hand is passed over a surface of a raised fabric having naps, in the opposite direction to the naps, the depth of color does not much change and increase.

Small — When one's hand is passed over a surface of a raised fabric having naps, in the opposite direction to the naps, color does not change.

## EXAMPLE 3

In Example 1, a 150 denier/40 filament wooly (false twisted) processed nylon yarn was used as warp and the following islands-in-sea type fiber whose sea component was a polyacrylonitrile, styrene copolymer (24, 76) and whose island component was nylon 6, was used as weft.

|    |                   |                |
|----|-------------------|----------------|
| 20 | Number of islands | 18             |
|    | Island/sea ratio  | 50/50          |
|    | Denier            | 4.8 d          |
|    | Fiber length      | 51 mm          |
|    | Number of crimps  | 8-12 mounts/in |

These yarns were made into 20/2 S spun yarns. (They were dyed in chestnut color with an acidic dyestuff.) The denier ratio Y of the weft to the warp was 1.75 and number of floating wefts U was 7.

Except for the foregoing, Example 1 was repeated to obtain a suede woven fabric which was anti-pilling and free from losing, and having excellent feel.

## EXAMPLE 4

On a raised woven fabric obtained by the same procedure as in Example 1, a dimethyl formamide solution of polyurethane (PU) obtained by an established method from polyether, polyester, methylene diphenyl diisocyanate and methylene-bis-aniline was coated in an amount of 9 g/m<sup>2</sup> calculated as PU from the back surface by a gravure coater having a gravure roll mesh No. 120. A raised woven fabric coated with an aqueous solution of polyurethane in an amount of 15 g/m<sup>2</sup> calculated as PU, was also prepared. When both of these fabrics were sufficiently dried at 140°C, they became 0.70 mm thick suede-like raised woven fabrics which were pliant (drapability 30 mm), having a better feel than the original, considerable balance between warp and weft, stabilized raised fibers (pilling resistance grade 3) and a much better long nap. But it was inferior to the fabric of Example 1. The original finished width of the fabric was 99.0 cm, after contraction, the width was 85.0 cm (a change of 14%). After removing the sea component, the width was 88.0 cm (a change of 11.1%); after dyeing, the width was 86.7 cm (a change of 12.4%); and after raising, the width was 77 cm (a change of 22.2%).

When each of these suede-like raised woven fabrics was observed under a scanning type electron microscope, it was confirmed that polyurethane adhered to the fiber of the fabric (except for the raised portion) in a dotted state, in a fibrous state or in a state of a plurality of small pieces of film.

## EXAMPLE 5

When a raised woven fabric was obtained by the same procedure as in Example 4 except using a warp, 150 denier/48 filament polyethylene terephthalate composite fibers having circular cross-sectional configuration of the bimetal type by difference in degree of polymerization (intrinsic viscosity values, 0.6 and 0.8),

pliant suede-like high-class raised woven fabrics having excellent raised fibers consisting of downy hair-like extra-fine fibers, with hardly conspicuous woven organization, and being free from losing, were obtained which were only a bit inferior to those of Example 1.

#### EXAMPLE 6

With an islands-in-sea type fiber consisting of 3.8 d  $\times$  51 mm and having a crimp at a ratio of 12 mounts/in consisting of 55% of polyethylene terephthalate as the island component and 45% of polystyrene as the sea component, a 2.5 d  $\times$  51 mm polyethylene terephthalate fiber containing 11 mol % of adipic acid as a copolymerization component was mixed at a ratio of 100 units of the former to 15 units of the latter, and the mixture was made into a 30/2 S spun yarn.

Next, using said spun yarn as weft and a 100 denier/32 filament wooly yarn of polyethylene terephthalate as warp, a 5-ply satin was woven at a density of 100 warps/in and 55 wefts/in. The denier ratio Y of the weft to the warp was 1.77 and number of floating wefts U was 4.

The obtained woven fabric was subjected to a heat treatment, from which the sea component was removed by trichloroethylene; thereafter, said fabric was dried and then dyed under pressure at 120°C in Midnight color (blue), and the dyed fabric was passed through a raising machine 8 times. The back-surface of the resulting raised woven fabric was slowly brought into contact with a hot roll at 235°C at a ratio of 0.5 m/min to partially melt said fabric. Thereafter, a partially laid portion of the raised fibers was buffed to stand them up again. The obtained raised woven fabric had drapeability of 28 mm, the feel of the warp and the weft was well balanced and said fabric had piling resistance of grade 5, which was very good.

The raised woven fabric was further treated with a 2% dimethyl formamide solution of polyurethane containing 10% of carbon black, coagulated, and dried. When said treated fabric was subjected to buffing, it became even better; having a feel close to that of suede.

When a section of this fabric was observed under a scanning type electron microscope, it was confirmed that the fiber of the fabric (except for the raised portion) was partially fused, and the polyurethane was adhered in a fine dotted state.

#### EXAMPLE 7

To a weft coming to the back surface was added a 100 denier/32 filament false-twisted processed yarn like that used as warp; a mix spun yarn of an islands-in-sea type fiber and a low-melting-point fiber the same as that in Example 5 was used as weft coming to the surface and a yarn the same as that in Example 6 was used as warp coming to the surface in weaving a double squeezed 5-ply satin. The denier ratio Y of the weft to the warp was 1.77 and number of floating wefts U was 4.

When the same treatment as in Example 4 was then carried out, a raised woven fabric having a better feel (warp and weft were well balanced) and excellent fixation of raised fibers (piling resistance grades 4 - 5) was obtained. Said fabric was excellent in its smoothness and chalk mark properties.

#### EXAMPLE 8

As in Example 6, for a low melting point fiber, a polypropylene fiber was used and the ratio thereof was made 18, parts. In addition, the step for dissolving polypropylene was carried out at a temperature within the range of 190° - 220°C.

The rest was done exactly as in Example 6. Although the base sheet of the raised fibers of the raised woven fabric looked whitish due to a dyed difference of polypropylene, it nonetheless had merchandisable interest in its own way, since said fabric had better fixation of the raised fibers (piling resistance grade 5) and excellent drapeability (32 mm) and feel. Warp and weft were excellent as compared with a raised fabric not added to a low melting point fiber of polypropylene.

The drapeability was determined by a cantilever method whereby a sample was caused to slide on a board inclined at 45° and the distance until it contacted a slope was measured. The pilling resistance was evaluated by the ICI pilling tester process in five grades.

#### EXAMPLE 9

As warp, a 75 denier/ 24 filament twin wooly yarn (false twisted processed yarn) of polyethylene terephthalate was used, and as weft, an islands-in-sea type composite fiber whose island component consisted of polyethylene terephthalate and whose sea component consisted of a polymer consisting mainly of polystyrene was used.

The particulars of the fiber used as weft were as follows:

|                                |              |
|--------------------------------|--------------|
| Number of islands              | 16           |
| Percentage of island component | 55%          |
| Percentage of sea component    | 45%          |
| Denier                         | 3.0 d        |
| Fiber length                   | 76 mm        |
| Number of crimp                | 12 mounts/in |

These fibers were made into 1/12 spun yarns (wool yarn counts) and twin processing was carried out (2/12). Using these yarns as warp and weft, respectively, a Turkish satin (4-ply satin) was woven so that the wearing density might become 75 warps/in and 37 wefts/in.

The denier ratio Y of the weft to the warp was 1.74 and number of floating wefts U was 3.

The obtained satin fabric was treated the same as in Example 1 to obtain a 0.78 mm thick suede-like raised woven fabric preferable for apparel having balanced warp and weft, excellent feel, excellent piling resistance, excellent nap without having any impression of the woven organization after dyeing.

#### EXAMPLE 10

Fibers the same as those in Example 9 were used and the weft was made into a 1/11 spun yarn.

These yarns were woven into a Turkish satin so that the weaving density might become 75 warps/in and 54 wefts/in. The denier ratio Y of the weft to the warp was 1.87 and number of floating wefts U was 3.

The satin fabric was efficiently washed with trichloroethylene 4 times to remove the sea component of the weft and thereafter said fabric was immersed in hot water at 96 - 98°C for 2 minutes to develop crimp of the warp.

The resulting treated fabric was passed through a French-style raising machine twice and a German-style raising machine twice, or a total of 4 times and thereafter through a shearing machine twice to obtain a raised woven fabric having excellent density of raised fibers in which the impression of the woven organization was not seen at all.

This raised woven fabric was immersed in and impregnated with a 7% DMF (dimethyl formamide) solution of polyurethane of the MBA series (MDI) using 75 parts of polyether glycol and 25 parts of polyester glycol. The impregnated fabric was squeezed at a clearance of 80% of the thickness of the fabric, wet coagulated and dried. The amount of polyurethane adhered to this dried fabric was 21 g/m<sup>2</sup>. Because the raised fibers on the surface of this fabric fell down remarkably, this fabric was passed through paper mesh No. 150 by a belt sander buffering machine to obtain a suede-like raised woven fabric having excellent feel, uniform nap, balanced warp and weft, and excellent piling resistance.

This suede-like fabric was dyed a deep red with a dispersed dyestuff by a circular pressuring dyeing machine, combined with an anti-static agent, made waterproof and made into a product.

The thickness of this treated fabric was 0.72 mm, said fabric being an excellent suede-like raised woven fabric excellent as apparel.

When a section of this product was observed under a scanning type electron microscope, a plurality of fine pieces of film of polyurethane adhered to the fiber of the fabric (except the raised portion) was observed.

#### EXAMPLE 11

Yarns the same as those in Example 1 were used and woven into a 5-ply satin fabric so that the wearing density might become 80 warps/in and 55 wefts/in.

The denier ratio Y of the weft to the warp was 1.75 and the number of floating wefts U was 4.

Said satin fabric was sufficiently washed with trichloroethylene 4 times to remove the sea component of the weft and then immersed in hot water at 96°–98°C for 2 minutes to develop crimp of the warp.

Next, the treated satin fabric was passed through a French-style raising machine 4 times and a German-style raising machine twice, or a total of 6 times to obtain a raised woven fabric having a high density of raised fibers in which the impression of the woven organization was not seen at all.

This raised fabric was impregnated with a 5% aqueous emulsion of polyurethane, squeezed so that the wet adhered amount of water-polyurethane might become 300 g/m<sup>2</sup>, passed through rolls, dried and solidified.

The obtained fabric had not as good a surface touch because the fibers of the raised portion fell down; however, when said fabric was passed through paper mesh No. 280 twice by a belt sander buffering machine to effect a buffering finish, the raised fibers became good.

The buffed fabric was then dyed in green with a dispersed dyestuff by a circular pressuring machine. After dyeing was carried out at 125°C for 1 hour and reduction washing was carried out at 80°C for 30 minutes, said fabric became a suede-like raised woven fabric having excellent feel, uniform nap, balanced warp and weft and excellent piling resistance.

When a section of this suede-like fabric was observed under a scanning type electron microscope, it was ob-

served that polyurethane adhered to the fiber of the fabric (except the raised portion) in a state of fine pieces of film.

#### EXAMPLE 12

Because some fuzz appeared on the back surface of the buffering-finished raised woven fabric obtained in Example 11, the back surface was passed through a fuzz burning machine and then dyed. Said fabric thus became a suede-like raised woven fabric having a smooth back surface and higher commercial value.

|            | Transverse cover factor           | Longitudinal cover factor        |
|------------|-----------------------------------|----------------------------------|
| 15         |                                   |                                  |
| Example 1  | $C = 60/\sqrt{20} \approx 13.4$   | $C = 100/\sqrt{35} \approx 16.9$ |
| Example 2  | $C \approx 13.4$                  | $C \approx 16.9$                 |
| Example 3  | $C \approx 13.4$                  | $C \approx 16.9$                 |
| Example 4  | $C \approx 13.4$                  | $C \approx 16.9$                 |
| Example 5  | $C \approx 13.4$                  | $C \approx 16.9$                 |
| Example 6  | $C = 55/\sqrt{30} \approx 10.05$  | $C = 100/\sqrt{53} \approx 13.7$ |
| Example 7  | $C \approx 10.05$                 | $C \approx 13.7$                 |
| Example 8  | $C \approx 10.05$                 | $C \approx 13.7$                 |
| Example 9  | $C = 37/\sqrt{20.3} \approx 8.22$ | $C = 75/\sqrt{35} \approx 12.7$  |
| Example 10 | $C = 54/\sqrt{18.7} \approx 12.5$ | $C = 75/\sqrt{35} \approx 12.7$  |
| Example 11 | $C = 55/\sqrt{20} \approx 12.3$   | $C = 80/\sqrt{35} \approx 13.5$  |
| 25         |                                   |                                  |
| Example 12 | $C \approx 12.3$                  | $C \approx 13.5$                 |

What is claimed is:

1. A suede-like raised woven fabric which comprises raised fibers covering the surface of said fabric and an elastic polymer impregnated throughout said fabric, wherein said fabric is woven and comprises warp and weft yarns, the weft of said fabric being a yarn consisting of a bundle of extra fine fibers, the mono-filament denier of which is 0.0001–0.4 denier, the warps of said fabric are yarns having a coil-like crimp capacity, the total denier of said warp yarn being 50–300 denier, and said raised fibers consisting mainly of said extra fine fibers which constitute said weft of said fabric.
2. The raised woven fabric according to claim 1 wherein said weft yarn is a thread.
3. The raised woven fabric according to claim 1 wherein said warp yarn having coil-like crimp capacity has a coil-like crimp.
4. The raised woven fabric according to claim 1 wherein said elastic polymer exists as a plurality of fine pieces of film in said fabric.
5. The raised woven fabric according to claim 1 wherein said elastic polymer exists in a fibrous state in said fabric.
6. The raised woven fabric according to claim 1 wherein said elastic polymer exists in a dotted state in said fabric.
7. The raised woven fabric according to claim 1 wherein said weft is a spun yarn consisting of said bundle of extra fine fibers.
8. The raised woven fabric according to claim 1 wherein said weft is a spun thread consisting of said bundle of extra fine fibers.
9. The raised woven fabric according to claim 1 wherein said warp is a false twisted processed yarn the mono-filament denier of which is 1–10 deniers.
10. The raised woven fabric according to claim 1 wherein said warp is a composite crimped yarn the mono-filament denier of which is 1–10 deniers.
11. The raised woven fabric according to claim 1 wherein said warp is a composite crimp thread the mono-filament denier of which is 1–10 deniers.

12. The raised woven fabric according to claim 1 wherein said weft is a single spun yarn having a size of 70-3,000 deniers.

13. The raised woven fabric according to claim 1 wherein said weft is a twin spun yarn having a size of 70-3,000 deniers.

14. The raised woven fabric according to claim 1 wherein said weft is a triple spun yarn having a size of 70-3,000 deniers.

15. The raised woven fabric according to claim 1 which satisfies the dual relationship:

$$30 \geq y > 1.4 \text{ and } U = 1 - 7;$$

wherein Y is the denier ratio of the weft to the warp and U is the number of floating wefts on the surface of said fabric.

16. The raised woven fabric according to claim 1 which satisfies the dual relationship:

$$1.4 \geq Y > 0.75 \text{ and } U = 3 - 12;$$

wherein Y is the denier ratio of the weft to the warp and U is the number of floating wefts on the surface of said fabric.

17. The raised fabric according to claim 1 wherein said fabric is a 4-ply satin.

18. The raised woven fabric according to claim 1 wherein said fabric is a 5-ply satin.

19. A process for the preparation of a suede-like raised woven fabric which comprises the following steps:

1. preparing a woven fabric from a weft consisting of a yarn consisting of a multi-core composite fiber in which the core components are surrounded by another component (sea component) the mono-filament denier of core component being 0.0001-0.4 denier, and a warp consisting of a yarn having coil-like crimp capacity;
2. removing the sea component from said weft;
3. impregnating throughout said fabric a solution of an elastic polymer in the obtained fabric;
4. drying to solidify said elastic polymer;
5. subjecting the surface of the obtained sheet to napping; and
6. developing the crimp at least once after said step of removing the sea component.

20. The process according to claim 19 wherein said weft yarn is a thread.

21. The process according to claim 19 wherein said sea component is a mix spun fiber.

22. The process according to claim 19 wherein said warp yarn having coil-like crimp capacity has coil-like crimp.

23. The process according to claim 19 wherein the impregnated solution of step 3 is an emulsion and its main medium is water.

24. The process according to claim 19 wherein the drying of step 4 is accomplished by wet coagulation.

25. The process for the preparation of a raised woven fabric according to claim 19 wherein said yarn capable of developing crimp is a potentially crimped composite fiber and said fabric is heated to develop crimp at least before imparting said elastic polymer to said fabric.

26. The process for the preparation of a raised woven fabric according to claim 25 wherein said development of crimp is effected at the same time with dyeing of said fabric.

27. The process for the preparation of a raised woven fabric according to claim 19 wherein said woven fabric

is raised before removal of said sea component of said weft.

28. The process for the preparation of a raised woven fabric according to claim 19 wherein said woven fabric is raised after removal of said sea component of said weft.

29. The process for the preparation of a raised woven fabric according to claim 19 wherein removal of said sea component of said weft is effected by immersing said woven fabric in a solvent for said sea component.

30. The process for the preparation of a raised woven fabric according to claim 19 wherein the concentration of said solution of said elastic polymer is 1-9% by weight.

31. The process for the preparation of a raised woven fabric according to claim 23 wherein the concentration of said emulsion of said elastic polymer is 1-9% by weight.

32. A process for the preparation of a suede-like raised woven fabric which comprises the following steps:

1. weaving a fabric whose weft is a yarn consisting of a multi-core type composite fiber wherein the core component is surrounded by another component (sea component) the mono-filament denier of said core component being 0.0001 - 0.4 denier and whose warp a coil-like crimp capacity;
2. raising the surface of said woven fabric;
3. impregnating a solution of an elastic polymer in said woven fabric throughout said fabric;
4. drying to solidify said elastic polymer; and
5. removing the sea component of said weft.

33. The process according to claim 32 wherein said weft yarn is a thread.

34. The process according to claim 32 wherein said sea component is a mix spun fiber.

35. The process according to claim 32 wherein said warp yarn having coil-like crimp capacity has a coil-like crimp.

36. The process according to claim 32 wherein the impregnated solution of step 3 is an emulsion and its main medium is water.

37. The process for the preparation of a raised woven fabric according to claim 32 wherein said yarn capable of developing a coil-like crimp is a potentially crimped composite fiber and said woven fabric is heated at least before said elastic polymer is imparted to said woven fabric to develop said crimp.

38. The process for the preparation of a raised woven fabric according to claim 37 wherein said development of crimp is effected at the same time with dyeing of said woven fabric.

39. The process for the preparation of a raised woven fabric according to claim 32 wherein said woven fabric is raised before removal of said sea component.

40. The process for the preparation of a raised woven fabric according to claim 32 wherein said woven fabric is raised after removal of said sea component.

41. The process for the preparation of a raised woven fabric according to claim 32 wherein removal of said sea component of said weft is effected by immersing said woven fabric in a solvent for said sea component.

42. The process for the preparation of a raised woven fabric according to claim 32 wherein the concentration of said solution of said elastic polymer is 1-9% by weight.

43. The process according to claim 42 wherein said solution is an emulsion.

44. The process for the preparation of a raised woven fabric according to claim 19 wherein said warp is a false twisted processed yarn.

45. The process for the preparation of a raised woven fabric according to claim 32 wherein said warp is a false twisted processed yarn.

46. The process for the preparation of a raised woven fabric according to claim 26 wherein the opposite surface of the surface subjected to napping is singed before dyeing of said fabric.

47. The process for the preparation of a raised woven fabric according to claim 26 wherein the opposite sur-

face of the surface subjected to napping is buffed before dyeing of said fabric.

48. The process for the preparation of a raised woven fabric according to claim 26 wherein the opposite surface of the surface subjected to napping is singed after dyeing of said fabric.

49. The process for the preparation of a raised woven fabric according to claim 26 wherein the opposite surface of the surface subjected to napping is buffed after dyeing of said fabric.

50. The process according to claim 32 wherein the solidification of step 4 is accomplished by wet coagulation.

\* \* \* \* \*

# REEXAMINATION CERTIFICATE (26th)

## United States Patent [19]

Okamoto et al.

[11] B1 3,865,678

[45] Certificate Issued Oct. 19, 1982

[54] SUEDE-LIKE RAISED WOVEN FABRIC AND PROCESS FOR THE PREPARATION THEREOF

[75] Inventors: Miyoshi Okamoto Osaka-fu; Shusuke Yoshida, Otsu; Tadashi Imai, Otsu; Tatsuo Watanabe, Otsu; Shinzo Nishikaku, Kusatsu, all of Japan

[73] Assignee: Toray Industries, Inc., Tokyo, Japan

### Reexamination Request

No. 90/000,123, Dec. 10, 1981

### Reexamination Certificate for:

Patent No.: 3,865,678

Issued: Feb. 11, 1975

Appl. No.: 338,962

Filed: Mar. 7, 1973

### [30] Foreign Application Priority Data

Mar. 7, 1972 Japan.....47-22766

Apr. 25, 1972 Japan.....47-40901

[51] Int. Cl.<sup>3</sup> ..... D04H 1/64; D04H 11/00; B29D 27/00

[52] U.S. Cl ..... 428/91; 428/96; 428/151; 428/259; 428/272; 428/371; 428/375; 428/369, 428/904; 139/37; 139/392; 139/420A

[58] Field of Search ..... 428/91; 96, 371, 904, 151, 428/259, 272, 375, 369; 139/37, 392, 420A

[56]

### References Cited

#### U.S. PATENT DOCUMENTS

|           |         |                    |         |
|-----------|---------|--------------------|---------|
| 3,050,821 | 8/1962  | Kilian.....        | 428/371 |
| 3,705,226 | 12/1972 | Okamoto et al..... | 428/96  |
| 3,986,331 | 10/1976 | Brumlik.....       | 428/371 |

#### FOREIGN PATENT DOCUMENTS

|          |         |                       |
|----------|---------|-----------------------|
| 2035669  | 1/1972  | Fed. Rep. of Germany. |
| 44-19282 | 8/1969  | Japan.                |
| 46-2782  | 1/1971  | Japan.                |
| 1300268  | 12/1972 | United Kingdom.       |

Primary Examiner—William J. Van Balen

[57]

### ABSTRACT

A suede-like raised woven fabric having raised fibers on the surface thereof; consisting mainly of a yarn or thread which consists of a bundle of extra-fine fibers (the monofilament denier of which is 0.0001–0.4 d). The preparation of the fabric comprises weaving, using as weft said yarn and using as warp a yarn having a coil-like crimp or a coil-like potential crimp capacity, in the organization of the woven fabric except for the raised portion, which consists of an elastic polymer dispersed and adhered in a fibrous state, and/or as fine pieces of film throughout the said fabric. Said fabric has a high density of suede-like naps, has excellent pilling resistance and, wrinkle resistance feel, and is suitable for apparel.



**REEXAMINATION CERTIFICATE  
ISSUED UNDER 35 U.S.C 307.**

NO AMENDMENTS HAVE BEEN MADE TO  
THE PATENT

AS A RESULT OF REEXAMINATION, IT HAS  
BEEN DETERMINED THAT:

5 The patentability of claims 1-50 is confirmed.

\* \* \* \* \*

10

15

20

25

30

35

40

45

50

55

60

65